

## UNITED STATES PATENT OFFICE

2,062,354

## CRYSTALLIZATION INHIBITOR FOR PARAFIN WAX IN LUBRICATING OILS

Garland H. B. Davis, Baton Rouge, La., assignor to Standard Oil Development Company, a corporation of Delaware

No Drawing. Application April 21, 1932,  
Serial No. 606,765

16 Claims. (Cl. 87—9)

The present invention relates to improved lubricating oils and more specifically to high grade lubricating oils obtained from wax-containing stocks characterized by relatively low solidification or congealing points. The invention will be fully understood from the following description of the new products and their method of manufacture.

In the production of high grade lubricating oils it is known that low solidification or pour point is desirable and at the same time it is recognized that wax-containing oils are highly desirable for lubricating quality. It is the present practice to remove wax from wax-containing oils by cold pressing or other low temperature means so as to produce paraffinic oils of low cold test. These methods are expensive and undesirable since they materially reduce the yield and quality of oil.

In a prior U. S. Patent 1,815,022 of July 14, 1931, it is disclosed that low pour oils can be produced from high pour stocks by the addition of certain pour inhibiting substances. The substances disclosed are of the class produced by the condensation of waxy hydrocarbons and aromatic hydrocarbons and have the peculiar property of preventing or inhibiting solidification of waxy oils at their normal temperatures, and thus enable them to pour at considerably lower temperatures.

The present invention relates to a similar condensation product having similar properties but which is clearly distinguished from the above product in that it is produced by condensation or polymerization of waxy hydrocarbons alone, in absence of aromatics or other cyclic hydrocarbons. In the practice of the invention waxy hydrocarbons which may be paraffin wax, montan wax, ceresin or hydrocarbon oils rich in such substances, are first treated so as to convert the waxy material into an active derivative capable of polymerization or condensation. For this purpose there are a variety of methods available of which the most desirable are those which do not substantially decompose the carbon structure of the wax; for example, the wax may be halogenated say by passing chlorine or bromine through the wax at a temperature of 200 to 300° F. This is preferably continued for 15 to 20 hours or more, so as to produce a derivative containing from about 10 to 15% of chlorine. The chlorinated or brominated waxy hydrocarbons may be polymerized by the action of catalysts of the type of aluminum chloride at low temperatures. About 3 to 10% of the anhydrous aluminum chloride, or

its equivalents such as the other aluminum halides or boron fluoride and similar known substances, is used, based on the weight of the chlorinated wax, and the temperature is from about room temperature to 150° F., and preferably below 125 or even 100° F. Low temperatures are made possible by the use of a high degree of agitation and this results in more powerful inhibitors. The time of condensation is from about 2 to 20 hours, but there is an optimum time depending on each set of conditions and it is most desirable to withdraw samples at intervals to determine the best time by actual test. During this reaction copious volumes of hydrochloric, or other halogen halide are evolved depending on the one used to halogenate the waxy hydrocarbon. Catalytic sludge is then separated from the oil, preferably by reaction with water or alkali in the manner described in the co-pending application, Serial Number 576,208, filed November 19, 1931, or it may be settled by long standing, or otherwise. The oil may then be treated in any convenient manner, for example, by washing with water, or alkali, or acid, or by clay filtration or the like, to produce a high grade refined product. Residual chlorine is generally low but it may be substantially completely eliminated by treating the oil with metallic sodium or mercury, or the like.

In the prior description the paraffin or other waxy hydrocarbon halides were used, but if desired partially dehydrogenated wax may be used and may be produced from the halide by gently heating to such a temperature as to cause the halogen halide to split from the hydrocarbon. This may be assisted by alkali, or metals such as zinc, or by catalytic halides such as barium, or calcium chloride. The temperature varies somewhat with the method used, but in general it is well below temperatures at which hydrocarbons decompose and in this way it is, therefore, possible to obtain a partial dehydrogenation, that is to say, to the extent of preferably not more than 1 molecule of hydrogen for each original hydrocarbon molecule without breaking the carbon to carbon linkages.

Other methods for dehydrogenating the wax or waxy hydrocarbons may also be used, and especially those like the one previously described, which do not decompose the carbon structure to any substantial extent and, therefore, do not give rise to complicated side reactions resulting in tar formation, are applicable.

If desired the olefin, or the halide as the case may be, may be concentrated before the poly-

merization or condensation step by any known methods, for example, by sweating the oily halide from the solid wax, or by use of suitable solvents which may have chemical or purely physical 5 action, but concentration is not required as the saturated wax does not interfere with the subsequent reaction. In fact, the wax or heavy viscous oil appears to be a valuable diluent and prevents agglomeration of the heavy condensed molecules 10 during reaction.

When using dehydrogenated wax, or other active derivatives of waxy hydrocarbons in place of the halogenated wax as described above, the condensation is carried out in substantially the 15 same manner and with substantially the same results. The proportion of the catalytic material, temperatures and time are substantially the same.

As an example of the present process the following may be considered:

20 Paraffin wax melting at about 122° F. is chlorinated by bubbling chlorine through the wax at a temperature of about 300° F. This is continued for about 20 hours when the product shows a content of about 12.2% chlorine. The chlor- 25 paraffin is then charged to a still and 5% of dehydrated barium chloride is added. The temperature is slowly raised to about 600° F. and then raised quickly to about 750° F. During this time large volumes of hydrochloric acid gas are 30 evolved but the carbonaceous material is otherwise substantially undecomposed. The material from the still is then transferred to an agitating vessel and an equal weight of paraffin wax is added, together with 5% by weight of anhydrous 35 aluminum chloride based on the original chlorinated paraffin. The mixture is then thoroughly agitated and heated gently to a temperature of 125° and held at this point for about 12 hours. At the end of this time about two-thirds of its 40 volume of kerosene is added and the catalyst sludge is allowed to slowly settle. The supernatant liquid is withdrawn, washed with water and distilled to remove the kerosene and a large part of the wax. The oil obtained has the following 45 characteristics:

|                         |                |
|-------------------------|----------------|
| Gravity                 | 29.8° A. P. I. |
| Saybolt vis. at 100° F. | 300 seconds    |
| Saybolt vis. at 210° F. | 234 seconds    |
| 50 Pour point           | 80° F.         |
| Flash point             | 620° F.        |
| Conradson carbon        | 1%             |

When 1% of the above material is added to a natural motor oil obtained from Pennsylvania 55 crude, and which has a natural pour point of 30° F. the pour point is reduced to 0° F. The inspection of the motor oil before and after the addition of 1% of the synthetic is as follows:

| 60                      | Original       |                | With 1 percent<br>of synthetic |
|-------------------------|----------------|----------------|--------------------------------|
| Gravity                 | 28.9° A. P. I. | 28.7° A. P. I. |                                |
| Saybolt vis. at 100° F. | 433 seconds    | 445 seconds    |                                |
| Saybolt vis. at 210° F. | 50 seconds     | 61 seconds     |                                |
| 65 Flash                | 445° F.        | 445° F.        |                                |
| Pour                    | 30° F.         | 0° F.          |                                |

The oils produced by the present method appear in most of their properties to be very similar to 70 the wax-base oils. The gravity is high in proportion to viscosity, the viscosity curve with temperature is relatively flat and the flash point is high in respect to viscosity. The oils are of good color, and are as stable to light, heat and oxidation as ordinary unblended oils, and do not in-

crease the tendency of oils containing the same to emulsify. They are characterized by substantially less residual carbon (Conradson carbon) than the oils produced by the method referred to previously, U. S. Patent 1,815,022, i. e. condensation of waxy hydrocarbons with aromatic hydrocarbons, and appear to be substantially equal to them in respect to pour inhibiting strength. For pour reduction the synthetic oil is added in proportion generally less than 10% and in almost 10 every case less than 5%. The strength of the pour inhibitor may vary somewhat according to the conditions of its manufacture, and the exact quantity used to produce a particular reduction in pour depends on its strength, as well as the susceptibility 15 of the oil. With distillate motor oils, spindle oils and the like it may be generally used in proportion of about 1% at which concentration there is a substantial pour reduction and only small or no substantial change in the ordinary physical 20 properties. The oils for pour reducing purposes are almost always more viscous than the oils with which they are blended and a slight increase in viscosity may often be observed. The lighter fractions of the synthetic product do not appear 25 to possess marked pour inhibiting strength and are often inactive. It is generally desirable to remove these fractions by reduction under vacuum maintaining the temperature below the cracking point to segregate the polymers of high 30 molecular weight for example above 1000 or 1200.

In the above description the pour point of the oil is determined by the standard test method given in the report on Petroleum Products and Lubricants and Methods for Tests Relating to 35 Petroleum Products by Committee D-2 of the American Association on Testing Materials published in 1928. The method appears on page 83 and the following pages of this report.

In the following claims the product is designed 40 as a polymerization product of waxy hydrocarbons, or of active derivatives obtained therefrom in absence of aromatic hydrocarbons. By these terms it is desired to include the reaction products obtained from the waxy hydrocarbon molecules through polymerization of any sort active derivatives thereof such as may be obtained by halogenation or partial dehydrogenation.

My invention is not to be limited by any theory 50 of the condensation or polymerization reactions, nor to the precise steps or method of preparation, but only by the following claims in which it is desired to claim all novelty inherent in the invention.

I claim:

1. Product according to claim 12 in which the synthetic is used in proportion below about 10%, effective substantially only for pour reduction.
2. Product according to claim 12 in which the synthetic is used in proportion below about 5%, effective substantially only for pour reduction.
3. Product according to claim 12 in which the synthetic is used in proportion in the order of 1%, effective substantially only for pour reduction. 65
4. Product according to claim 12 in which the synthetic is obtained by polymerization of a waxy hydrocarbon containing from about 10 to 15% by weight of a halogen.
5. Product according to claim 12 in which the synthetic is obtained by polymerization of a partially dehydrogenated waxy hydrocarbon of the type produced by chlorination to 10 to 15% by weight of chlorine and then dechlorinating.
6. An improved lubricating oil of low cold test 75

comprising a normally higher cold test oil blended with a small quantity, in the order of 1%, of a high molecular weight hydrocarbon of the type produced by low temperature aluminum chloride polymerization of chlorinated paraffin in absence of cyclic materials.

7. Product according to claim 6 in which the synthetic is of the type produced from paraffin wax containing 10-15% of chlorine.

10 8. An improved lubricating oil of low cold test comprising a normally higher cold test oil blended with a small quantity in the order of 1% of a high molecular weight hydrocarbon of the type produced by low temperature aluminum chloride polymerization of a partially dehydrogenated paraffin wax of the type obtained by chlorination to 10 to 15% by weight of chlorine and then dechlorinating in absence of cyclic material.

9. Product according to claim 8 in which the synthetic is of the type produced by polymerization of paraffin wax dehydrogenated without decomposition of the carbon structure.

10. Product according to claim 12 in which the polymerization product is prepared at temperatures of the order of room temperature to about 150° F.

11. An improved lubricating oil of low cold test comprising a wax-containing oil and a synthetic hydrocarbon formed by the polymerization in absence of cyclic materials and at a temperature below that at which decomposition occurs, of an active derivative of a waxy hydrocarbon of

the same carbon structure as the said waxy hydrocarbon, the synthetic being in pour reducing proportion.

12. An improved lubricating oil of low pour point comprising a wax-containing oil and a synthetic polymer of an uncracked waxy hydrocarbon, prepared by condensation thereof in absence of cyclic materials at a temperature below the decomposing temperature of the wax, said polymer being in small amount whereby the pour point of the waxy oil is reduced.

13. An improved lubricating oil comprising a blend of a viscous hydrocarbon oil containing waxy constituents in proportion to give it a relatively high pour point, and a synthetic hydrocarbon prepared by polymerization in the absence of cyclic materials and at a temperature below that at which decomposition occurs, of an active derivative of a waxy hydrocarbon of the same carbon structure as the said waxy hydrocarbon, the synthetic being in pour reducing proportion.

14. Composition according to claim 13 in which the said synthetic has a molecular weight above 1000.

15. Composition according to claim 11 in which said active derivative is a halogenated wax.

16. Composition according to claim 11 in which said active derivative comprises a mixture of olefines prepared by dehydrogenation of paraffine wax.

GARLAND H. B. DAVIS.